

## UNITED STATES PATENT OFFICE

2,521,908

## 1-HYDROXY-2-NAPHTHAMIDE COLORED COUPLERS

Dudley B. Glass, Paul W. Vittum, and Arnold Weissberger, Rochester, N. Y., assignors to Eastman Kodak Company, Rochester, N. Y., a corporation of New Jersey

No Drawing. Application March 13, 1947,  
Serial No. 734,548

10 Claims. (Cl. 95—6)

**1** This invention relates to color photography and particularly to color couplers for use in photographic processes.

Color-forming compounds which react with the development product of aromatic amino developing agents to form colored images upon photographic development are well known. Generally, these color-forming compounds of couplers are colorless or substantially colorless. This lack of color is usually desirable where the coupler is to be incorporated in the emulsion layer and the unused coupler remains after formation of the colored image. When the coupler is used in the developing solution, it may be colored without detriment to the final image and certain colored couplers have been used in this way.

In our prior application Serial No. 533,931, filed May 3, 1944, now Patent No. 2,455,169, of which the present application is a continuation-in-part, we have described couplers having the general formula:



in which R is a benzene or naphthalene nucleus which has the azo group in a position para to the hydroxyl group and R' an aromatic or heterocyclic radical. These couplers are in themselves more or less strongly colored and during the coupling reaction, the chromophore system in the coupler is destroyed or split off with the result that the original color of the coupler is destroyed and a new dye is formed upon coupling. Thus on developing an emulsion layer containing one of these colored couplers, the coupler color is destroyed and a new color is formed by the coupling reaction at those points where development occurs. There is formed in this way a dye image of one color on a background of another color.

We have now found a class of colored couplers of the general structure described in our prior application Serial No. 533,931 which possess valuable properties for purposes of color photography. These couplers react in the same way as those described in our prior application to form a new dye on coupling by destruction or replacement of the chromophoric group but possess additional valuable properties with respect to the color of the image dye and the ease of coupling. All of these compounds are yellow

**2** to orange-red in color and yield cyan or blue-green dyes by reaction with the oxidized developing agent.

The couplers which we propose to use according to the present invention have the following general formula:



in which X is hydrogen or alkyl, Y is a mononuclear aryl radical, such as a mononuclear aryloxyphenyl radical, or an aralkyl radical, and R is a mononuclear aryl radical. By "mononuclear aryl" we mean an aryl radical of the benzene series, that is, a single aryl ring which may contain substituents.

In the general formula X may be a hydrogen atom or an alkyl radical such as methyl, ethyl, propyl, butyl or amyl; Y may be an aryl radical especially a mononuclear aryl radical such as phenyl or substituted phenyl, a mononuclear aryloxyphenyl radical such as p-tertiary-butyl-30 phenoxyphenyl, p-tert.-amylphenoxyphenyl, 2,4-diamylphenoxyphenyl or phenoxyphenyl or an aralkyl radical such as benzamidophenethyl or 4-[2-(2,4-diamylphenoxy)-5-(3,5-dichlorosulfonylbenzamido)benzamido]phenethyl and R is 35 a mononuclear aryl radical such as phenyl, o-methoxyphenyl, acetylaminophenyl, o-methoxy-p-nitrophenyl, o-methoxyphenylazo, o-methoxyphenyl, p-bromophenyl, or o-carbethoxyphenyl.

40 In each case the position para to the phenolic hydroxyl group of the coupler, which is the reactive position of the coupler, is substituted with an azo group and this group is split off or removed by the oxidized developer when the azo-substituted coupler is treated with the oxidized developer either in aqueous solution or in the photographic emulsion layer. Thus the coupler may be converted to a differently colored compound and the azo group readily removed from it by means of reaction with the oxidized de-

veloping agent. The reaction appears to proceed as follows:



The following examples illustrate compounds which may be used according to our invention:

1. 15 1-hydroxy-4-(p-phenylazophenoxy)-2-naphthalen-1-yl acetate
2. 20 1-hydroxy-4-(o-methoxyphenylazo)-4'-(p-tert.-butylphenoxy)-2-naphthalen-1-yl acetate
3. 25 1-hydroxy-4-(p-acetamidophenylazo)-4'-(p-tert.-butylphenoxy)-2-naphthalen-1-yl acetate
4. 30 1-hydroxy-4-(2-methoxy-4-nitrophenylazo)-4'-(p-tert.-butylphenoxy)-2-naphthalen-1-yl acetate
5. 35 1-hydroxy-4-(o-methoxyphenylazo)-4'-(2,4-diamylphenoxy)-2-naphthalen-1-yl acetate
6. 40 1-hydroxy-4-(p-bromophenylazo)-4'-(2,4-diamylphenoxy)-2-naphthalen-1-yl acetate
7. 45 1-hydroxy-4-(p-bromophenylazo)-4'-(2,4-diamylphenoxy)-2-naphthalen-1-yl acetate
8. 50 1-hydroxy-4-phenylazo-N-[4-[2-(2,4-diamylphenoxy)-5-(3,5-dichlorosulfonylbenzamido)benzamido]phenethyl]-2-naphthamide
9. 55 1-hydroxy-4-(o-carbethoxyphenylazo)-N-methyl-2-naphthalen-1-yl acetate
10. 60 1-hydroxy-4-(o-carbethoxyphenylazo)-N-methyl-2-naphthalen-1-yl acetate
11. 65 1-hydroxy-4-(o-carbethoxyphenylazo)-N-methyl-2-naphthalen-1-yl acetate
12. 70 1-hydroxy-4-(o-carbethoxyphenylazo)-N-methyl-2-naphthalen-1-yl acetate
13. 75 1-hydroxy-4-(o-carbethoxyphenylazo)-N-methyl-2-naphthalen-1-yl acetate

- 10.
- 1-hydroxy-4-phenylazo-N-isoamyl-2-naphthylidene
- 11.
- 1-hydroxy-4-(2-methoxy-4-nitrophenylazo)-N-isoamyl-2-naphthylidene
- 12.
- 1-hydroxy-4-[2-methoxy-4-(o-methoxyphenylazo)-phenylazo]-N-isoamyl-2-naphthylidene

Our compounds may be incorporated either in the developing solution or in the emulsion layer according to their intended use and diffusion characteristics. Generally, they will be used in one of the emulsion layers of a multi-layer coating in order to secure the masking effects described in Hanson U. S. application Serial No. 533,910, filed May 3, 1944, now Patent No. 2,449,966. The Hanson process involves a color correction method in which a color coupler is incorporated in the photographic emulsion layer prior to exposure and upon development is converted to a colored image where the layer is exposed. The coupler remaining in the unexposed portions of the layer retains its original color and by suitable choice of the color of the original coupler and the color of the final dye image, a masking or correction effect can be obtained.

The compounds employed according to our invention may be prepared by any suitable method such as by reaction of the naphthamide with the appropriate diazonium compound. For example, compound No. 1 was prepared as follows:

1. 1-hydroxy-4'-(p-tert.-butylphenoxy)-2-naphthylidene was prepared by the condensation of equi-molecular quantities of phenyl 1-hydroxy-2-naphthoate and p-(p-tert.-butylphenoxy)-aniline at 200° for one hour. The product was purified by recrystallization from a mixture of benzene and ligroin.

The p-(p-tert.-butylphenoxy)-aniline was prepared by alkali condensation of hot p-nitro-chlorobenzene and p-tert.-butylphenol followed by catalytic reduction of the nitro compound in the presence of Raney nickel.

1-hydroxy-4-phenylazo-4'-(p-tert.-butylphenoxy)-2-naphthylidene (1) was prepared by adding an aqueous solution of 1.05 moles of benzene diazonium chloride to one mole of 1-hydroxy-4'-(p-tert.-butylphenoxy)-2-naphthylidene dissolved in eight liters of pyridine-ethanol (1-1) solution at 5° C. The product is isolated by pouring the mixture into an excess

of dilute hydrochloric acid. The pure dye is obtained by crystallization from dioxane or acetic acid.

Compounds 2 to 5 were prepared in the same manner as compound 1 using the following couplers and diazonium salts.

| Dye No. | Coupler                                              | Diazonium salt                                   |
|---------|------------------------------------------------------|--------------------------------------------------|
| 10.     |                                                      |                                                  |
| 2.      | 1-hydroxy-4'-(p-tert.-butylphenoxy)-2-naphthylidene. | o-methoxybenzene diazonium chloride.             |
| 3.      | 1-hydroxy-4'-(p-tert.-butylphenoxy)-2-naphthylidene. | p-acetamido benzene diazonium chloride.          |
| 4.      | 1-hydroxy-4'-(p-tert.-butylphenoxy)-2-naphthylidene. | 2-methoxy-4-nitrobenzene diazonium chloride.     |
| 15.     |                                                      |                                                  |
| 5.      | 1-hydroxy-4'-(p-tert.-butylphenoxy)-2-naphthylidene. | 2-methoxy-4-phenylazobenzene diazonium chloride. |

Compound No. 6 was prepared as follows:

20. 1-hydroxy-4'-(p-tert.-amylphenoxy)-2-naphthylidene was prepared by the condensation at room temperature of one equivalent of 1-hydroxy-2-naphthoyl chloride with two equivalents of 4-(p-tert.-amylphenoxy)aniline in ether. The amine hydrochloride was removed by filtration and the filtrate was concentrated to a crude product which was recrystallized from a mixture of ligroin and benzene.

The 4-(p-tert.-amylphenoxy)aniline was prepared by the condensation of hot p-nitrochlorobenzene and p-tert.-amylphenol in alkali to yield 4-(p-tert.-amylphenoxy)nitrobenzene. The nitro compound was reduced catalytically in the presence of Raney nickel to 4-(p-tert.-amylphenoxy)aniline.

35. 1-hydroxy-4-(o-methoxyphenylazo)-4'-(p-tert.-amylphenoxy)-2-naphthylidene (6) was prepared by adding an equivalent solution of 1.05 mols of o-methoxybenzene diazonium chloride to 40. 1 mol of 1-hydroxy-4'-(p-tert.-amylphenoxy)-2-naphthylidene in 8 liters of pyridine ethanol (1:1) solution at 5° C. The product was isolated by pouring the mixture into an excess of hydrochloric acid. The pure dye was obtained by crystallization from dioxane or acetic acid.

45. Compound No. 7 was prepared as follows:

50. 1-hydroxy-4'-(2,4-diamylphenoxy)-2-naphthylidene was prepared in a manner similar to 1-hydroxy-4'-(p-tert.-butylphenoxy)-2-naphthylidene, which was used in the preparation of compound No. 1, by using p-(2,4-diamylphenoxy)aniline instead of p-(p-tert.-butylphenoxy)aniline.

55. 1-hydroxy-4-(p-bromophenylazo)-4'-(2,4-diamylphenoxy)-2-naphthylidene was prepared by treating 1-hydroxy-4'-(2,4-diamylphenoxy)-2-naphthylidene with p-bromobenzene diazonium chloride.

60. Compound No. 8 was prepared in the following manner:

65. 8. 1-hydroxy-N-[2-(2,4-diamylphenoxy)-5-(3,5-dichloro-sulfamylbenzamido)benzamido]phenethyl)-2-naphthamide was prepared by the following steps:

65. (a) Phenyl 1-hydroxy-2-naphthoate was condensed at 150° for one-half hour with an equimolecular quantity of p-nitrophenethylamine yielding 1-hydroxy-N-(p-nitrophenethyl)-2-naphthamide.

70. (b) The nitro compound was reduced catalytically in the presence of Raney nickel to the amine.

(c) 1-hydroxy-N-(p-aminophenethyl)-2-naphthamide was condensed in acetic acid and 75. sodium acetate at room temperature with an

equimolecular quantity of 2 - (2,4 - diamylphenoxy) - 5 - nitrobenzoyl chloride.

(d) 1-hydroxy-N-{4-[2-(2,4-diamylphenoxy)-5-aminobenzamido]phenethyl}-2-naphthamide was prepared by the catalytic reduction in the presence of Raney nickel of the nitro compound obtained in step (c).

(e) 1 - hydroxy - N - {4 - [2 - (2,4 - diamylphenoxy) - 5 - (3,5-dichlorosulfonylbenzamido) - benzamido]phenethyl}-2-naphthamide was prepared by the condensation of an equimolecular quantity of 3,5-dichlorosulfonyl benzoyl chloride and the amine of step (d) in dioxane and quinoline.

The final compound was prepared by the simple treatment of 1 - hydroxy-N-{4-[2-(2,4-diamylphenoxy) - 5-(3,5-dichlorosulfonylbenzamido) - benzamido]phenethyl}-2-naphthamide with benzene diazonium chloride.

Compound 9 was prepared by the condensation in ether of two equivalents of N-methylaniline with 1 equivalent of 1-hydroxy-2-naphthoyl chloride to produce 1-hydroxy-N-methyl-2-naphthanilide. The final compound was prepared by treating this intermediate with o-carboxybenzene diazonium chloride.

Compound 10 was prepared by the condensation in ether of 2 equivalents of N-isoamylaniline with 1 equivalent of 1-hydroxy-2-naphthoyl chloride to produce 1-hydroxy-N-isoamyl-2-naphthanilide. This intermediate was treated with benzene diazonium chloride to produce the final compound.

Compounds 11 and 12 were prepared similarly to compound 10 by treating 1-hydroxy-N-isoamyl-2-naphthanilide with the appropriate diazonium salt as follows:

| Dye No. | Coupler                              | Diazonium salt                                                |
|---------|--------------------------------------|---------------------------------------------------------------|
| 11..... | 1-hydroxy-N-isoamyl-2-naphthanilide. | 2-methoxy-4-nitrobenzene diazonium chloride.                  |
| 12..... | 1-hydroxy-N-isoamyl-2-naphthanilide. | 2-methoxy-4-(o-methoxyphenyl-azo) benzene diazonium chloride. |

Various photographic developing agents can be employed with the couplers of our invention. The primary aromatic amino developing agents are generally suitable including the phenylenediamines and aminophenols. The alkyl phenylenediamines may be substituted in the amino group as well as in the ring. Suitable compounds are diethyl paraphenylenediamine, monomethyl paraphenylenediamine, dimethyl paraphenylenediamine and para-aminophenol. These compounds are usually employed in the salt form, such as the hydrochloride or the sulphate which are more stable than the free amines. All of these compounds have a primary amino group which enables the oxidation product of the developer to couple with the color-forming compounds to form dye images.

The following developing solution is suitable for developing gelatino silver halide layers containing colored couplers according to our invention.

|                                          | Grams |
|------------------------------------------|-------|
| 2-amino-5-diethyl-amino toluene HCl..... | 2     |
| Sodium sulphite.....                     | 2     |
| Sodium carbonate.....                    | 20    |
| Potassium bromide.....                   | 2     |
| Water to 1 liter.                        |       |

It will be understood that the examples and modifications set forth herein are illustrative only and that our invention is to be taken as limited only by the scope of the appended claims.

We claim:

1. The method of developing a colored image in a silver halide emulsion layer which comprises exposing said emulsion layer and developing it with a primary aromatic amino developing agent in the presence of a coupler compound having the formula:



where X is selected from the class consisting of hydrogen and alkyl radicals, Y is selected from the class consisting of mononuclear aryl radicals and aralkyl radicals and R is a mononuclear aryl radical.

2. The method of developing a colored image in a silver halide emulsion layer which comprises incorporating in said layer a coupler compound having the formula:



40 where X is selected from the class consisting of hydrogen and alkyl radicals, Y is selected from the class consisting of mononuclear aryl radicals and aralkyl radicals and R is a mononuclear aryl radical, exposing said layer and developing it with a primary aromatic amino developing agent, thereby splitting off the  $-\text{N}=\text{N}-\text{R}$  group in said coupler compound and coupling said compound at the point of splitting with the oxidation product of the primary aromatic amino developing agent to form a dye image.

3. The method of developing a colored image in a silver halide emulsion layer which comprises incorporating in said layer a coupler compound having the formula:



65 where Y is a mononuclear aryl-oxyphenyl radical and R is a mononuclear aryl radical, exposing said layer and developing it with a primary aromatic amino developing agent, thereby splitting off the  $-\text{N}=\text{N}-\text{R}$  group in said coupler compound and coupling said compound at the point of splitting with the oxidation product of the primary aromatic amino developing agent to form a dye image.

4. The method of developing a colored image 75 in a silver halide emulsion layer which comprises

9

incorporating in said layer a coupler compound having the formula:



exposing said layer and developing it with a primary aromatic amino developing agent, thereby splitting off the



group in said coupler compound and coupling said compound at the point of splitting with the oxidation product of the primary aromatic amino developing agent to form a dye image.

5. The method of developing a colored image in a silver halide emulsion layer which comprises incorporating in said layer a coupler compound having the formula:



exposing said layer and developing it with a primary aromatic amino developing agent, thereby splitting off the



group in said coupler compound and coupling said compound at the point of splitting with the oxidation product of the primary aromatic amino developing agent to form a dye image.

6. A gelatino silver halide emulsion layer containing a coupler compound having the formula:



where X is selected from the class consisting of hydrogen and alkyl radicals, Y is selected from the class consisting of mononuclear aryl radicals, aralkyl radicals and R is a mononuclear aryl radical.

7. A gelatino silver halide emulsion layer containing a coupler compound having the formula:



where Y and R are mononuclear aryl radicals.

10

8. A gelatino silver halide emulsion layer containing a coupler compound having the formula:



15 where Y is a mononuclear aryloxyphenyl radical and R is a mononuclear aryl radical.

9. A gelatino silver halide emulsion layer containing a coupler compound having the formula:



30 10. A gelatino silver halide emulsion layer containing a coupler compound having the formula:



DUDLEY B. GLASS.  
PAUL W. VITTM.  
ARNOLD WEISSBERGER.

#### REFERENCES CITED

50 The following references are of record in the file of this patent:

#### UNITED STATES PATENTS

| Number    | Name         | Date          |
|-----------|--------------|---------------|
| 2,189,817 | Morris       | Feb. 13, 1940 |
| 2,220,123 | Schwarz      | Nov. 5, 1940  |
| 2,310,943 | Dorough      | Feb. 16, 1943 |
| 2,313,586 | Salminen     | Mar. 9, 1943  |
| 2,324,832 | Frohlich     | July 20, 1943 |
| 2,357,394 | Frohlich     | Sept. 5, 1944 |
| 2,455,169 | Glass et al. | Nov. 30, 1948 |

#### FOREIGN PATENTS

| Number     | Country       | Date          |
|------------|---------------|---------------|
| 65 519,208 | Great Britain | Mar. 19, 1940 |